

3,501,373  
DE-INKING WASTE PRINTED CELLULOSIC STOCK

Robert H. Illingworth, Madison, N.J., assignor to Garden State Paper Co. Inc., Garfield, N.J., a corporation of Delaware

No Drawing. Continuation-in-part of application Ser. No. 193,448, May 9, 1962. This application Nov. 4, 1966, Ser. No. 591,972

Int. Cl. D21c 5/02

U.S. Cl. 162—5

15 Claims

## ABSTRACT OF THE DISCLOSURE

This invention provides an improved method of de-inking waste printed paper. The improved method comprises utilizing as the de-inking agent in aqueous solution a small effective amount of non-ionic surface active agent and a hydrocarbon component, the non-ionic surface active agent corresponding to the formula



wherein R represents the residue of an alkyl phenol in which the total number of carbon atoms is between 7 and 24, R<sup>1</sup> represents hydrogen or lower alkyl, and n is an integer of from 2 to 100, and the hydrocarbon component being an aliphatic hydrocarbon having a boiling point above about 100° F. and a melting point below about 40° F. or a chlorinated aromatic hydrocarbon having at least one chlorine atom attached to an aromatic carbon atom the weight ratio of non-ionic surface active agent to hydrocarbon component being between 10:1 and 1:10.

## COPENDING APPLICATION

This application is a continuation-in-part of my copending application Ser. No. 193,448, issued as U.S. Patent 3,446,696, on May 9, 1969.

This invention relates to improvements in de-inking printed waste cellulosic stock.

It is an object of the present invention to provide improved methods and agents for de-inking printed cellulosic material to produce a pulp that can be readily and economically handled on conventional paper making machines to produce newsprint, magazine or book stock.

It is another object of this invention to provide improved processes and agents for de-inking waste printed paper to produce a pulp at least substantially equal, and often superior, in brightness, color and strength to that of virgin pulp.

Still another object of this invention is to provide improved agents and methods capable of de-inking a wide variety of waste printed paper, regardless of the type of ink or method of printing originally employed to produce the printed paper.

Other objects of the present invention will in part be clear and will in part appear hereinafter.

Commercial conversion of waste newspaper, magazine and other types of printed waste cellulosic stock to a pulp capable of re-use in forming paper or other cellulosic products has been a much sought after goal in the paper industry.

Although many processes for de-inking such printed cellulosic material have been heretofore proposed, in general, these have not proved commercially satisfactory. Many of these processes, for example, when tested on a commercial scale with the general run of waste newspaper and junk, fail to yield a pulp suitable for re-use as newsprint, magazine or book stock. The failure may be attributable to the fact that many of these processes drive a significant portion of the ink particles into the cellulosic

fibers, thereby rendering the pulp gray and unsatisfactory for use except for the manufacture of low grade paper materials, for example, low grade packaging cartons. Other of these processes are so expensive, time-consuming, laborious and complicated that they are simply not economically feasible.

In co-pending applications there are described processes for de-inking waste newspaper, magazine and other types or printed waste cellulosic stock which utilize, as the active de-inking agent, certain non-ionic detergents, e.g., ethylene oxide adducts of alkyl phenols.

Such non-ionic detergents, by themselves, give satisfactory de-inking results when used with the general run-of-the-mill waste newspaper and magazine stock produced; for example, standard planographic, e.g., off-set, printing techniques and inks. With certain waste printed cellulosic stock, however; e.g., paper printed by intaglio such as rotogravure techniques and inks, non-ionic detergents of the type specified above and in the co-pending 20 applications do not, by themselves, accomplish a completely satisfactory de-inking job.

As will be readily apparent, in commercial de-inking, it would be highly advantageous if the process would be able to handle a wide variety of waste printed stock, regardless of the type of ink or printing technique originally used in producing the waste printed paper. Otherwise, a costly and time-consuming paper separation step would have to precede de-inking. The economics of paper de-inking are such that a paper separation or classification 30 step could well spell the difference between success and failure.

According to the present invention, it has been discovered that improved de-inking results may be realized by utilizing as the active de-inking agent the combination of (1) a non-ionic detergent, and (2) a hydrocarbon component which can be either an aliphatic hydrocarbon or a chlorinated aromatic hydrocarbon.

This combination of ingredients, when used as described herein, has been found to be effective in de-inking 40 all types of waste printed cellulosic stock, regardless of the type of ink or printing technique originally utilized in producing the paper. The combination is particularly advantageous in that it results in increased brightness of the de-inked stocks and permits greater versatility of processing. Thus, the stock to be de-inked can be added to the aqueous de-inking composition either before or after the aforesaid combination of ingredients is added. Alternatively, the paper can be added to the reactor before addition of water and de-inking ingredients. As a further advantage, freshly printed newspaper, i.e., "over-issue news," can be treated immediately without the formation or retention of ink spots or smudges.

The aliphatic hydrocarbon can be saturated or unsaturated but preferably will be substantially saturated. It is also preferably a liquid under the operating conditions. Normally this will be at room temperature. Hence it is preferred that the aliphatic hydrocarbon have a melting point or range below about 40° F. and an initial boiling point or range above about 100° F. and more preferably above about 110° F. There can be employed a mixture of aliphatic hydrocarbons such as is present in various petroleum distillates. When such mixtures are used, the melting and boiling points or ranges specified above are those attributable to the entire mixture. Within this category are such products as solvent naphthas, kerosene, gasoline and alkanes meeting the requirements such as the several isomeric heptanes, octanes and nonanes.

The chlorinated aromatic hydrocarbon should preferably be a liquid under the operating conditions, should be monocyclic and should have at least one chlorine atom attached to an aromatic carbon atom. It is preferred that

non-aromatic substituents be avoided except that a single alkyl group having up to four carbon atoms can be a substituent on the aromatic nucleus and in addition, a methyl group may also be present. Thus the chlorinated aromatic hydrocarbon can have the structure



wherein the R groups are selected from among chlorine, alkyl having 1 to 4 carbon atoms and hydrogen, at least one R group being chlorine, up to a total of six chlorine substituents, not more than one R being alkyl, except that a second R may be methyl. In the preferred embodiment, there are from one to three chlorine substituents, and all other R groups are hydrogen.

Mixtures of several chlorinated aromatic hydrocarbons meeting the foregoing requirements can be employed, such as a mixture of mono-, di-, and trichlorobenzenes.

Representative chlorinated aromatic hydrocarbons that can be employed either alone or in mixtures with each other, include chlorobenzene; 1,3-dichlorobenzene; 1,3,5-trichlorobenzene; ortho-chlorotoluene, para-chlorotoluene; para-chloroethylbenzene.

The non-ionic detergents suitable for use may be described as water-soluble synthetic non-ionic surface active agents containing a polyoxyalkylene chain of at least two alkenoxy groups, and derived from alkyl phenolic compounds in which the total number of alkyl carbon atoms is between 4 and 24.

The above defined non-ionic surface active agents operative in the instant invention may be more specifically represented by the general formula



wherein R represents the residue of a suitable alkyl phenol, R<sup>1</sup> represents hydrogen or lower alkyl, and n has a value from 2 to 100 or more and usually from about 4 to 30. Compounds of this type are well known in the art and are disclosed along with suitable methods for their preparation in U.S. Patent 2,946,921. In general, they may be obtained by condensing a polyglycol ether containing the required number of alkenoxy groups or an alkylene oxide such as propylene oxide, butylene oxide, or preferably ethylene oxide, with a suitable alkyl phenol. The amount of alkylene oxide condensed with the alkyl phenol, i.e., the length of the polyoxyalkylene chain, will depend primarily upon the particular compound with which it is condensed. As a convenient rule of thumb, approximately 1 mole of alkylene oxide should be employed for each two carbon atoms in the alkyl phenol. However, the optimum amount of alkylene oxide may readily be determined in any particular case by preliminary test and routine experimentation.

An especially suitable non-ionic detergent is an ethylene oxide adduct of dodecylphenol having a formula corresponding to that indicated above, wherein n is between about 8 and 15. Another particularly suitable non-ionic detergent is a condensation product of nonyl-phenol and ethylene oxide having the structural formula



wherein n is an integer between 8 and 15.

The amounts of non-ionic detergent and aliphatic hydrocarbon or aromatic chlorinated hydrocarbon employed should be carefully controlled. Based on the weight of paper, the amount of each of these materials may vary between about 0.1 and 3.0 percent. Especially good results are obtained when about 0.5 to 1 percent by weight of paper of each material is employed, and this amount is preferred.

The relative proportion of the non-ionic detergent to

the hydrocarbon component may be varied over fairly wide ranges. In general, the weight ratio of non-ionic detergent to hydrocarbon component may vary from about 10:1 to 1:10, but preferably it is about 1:1 to 1:2.

Preferably, the non-ionic detergent and hydrocarbon component are admixed, and the admixture added to water to form the de-inking solution.

The combined de-inking agent constitutes a part of the present invention, and, as indicated above, comprises compositions satisfying the following formula:

Parts by wt.

|                       |       |      |
|-----------------------|-------|------|
| Non-ionic detergent   | ----- | 10-1 |
| Hydrocarbon component | ----- | 1-10 |

15 The temperature of the de-inking solution may vary anywhere from room temperature, e.g., 40° to 70° F., up to the cloud point or volatilization temperature of the non-ionic detergent, or the hydrocarbon component, whichever is the lower, although preferably the de-inking solution is employed at room temperature.

20 Best results are achieved with the de-inking solutions described herein when they are alkaline in pH and it therefore is desirable that an alkali be included therein. Although any suitable alkali or alkaline earth metal hydroxide or salt may be employed, the alkali metal hydroxides and salts, such as sodium hydroxide, potassium hydroxide, soda ash and the like are preferred. Enough of the alkali should be added to maintain the pH of the de-inking solution between about 7.0 and 11, or even 30 higher, and preferably at least about 7.1.

25 In preparing the de-inking solution, water is charged to the reactor or pulper and the active de-inking agents described hereinabove added. The de-inking agents are preferably added to the water prior to the addition of the wastepaper.

30 To the resulting solution is added the printed paper, scrap or junk. Alternately, the printed paper, scrap or junk can be added to the reactor or pulper in the dry state followed by addition of water and de-inking agents in either order or as a mixture. The printed cellulosic charge may, if desired, be shredded by appropriate means prior to treatment. This, however, is not necessary, and the waste material may be treated without shredding or without any subdivision in size whatsoever. It is one of the advantages of this invention that costly shredding or pulping techniques prior to de-inking need not be employed. Thus, the waste material to be de-inked is preferably added to the treating solution in its naturally dry condition, i.e., without being subjected to moisture or water other than that which is normally present in the atmosphere or 45 the waste material can, if desired, be wet or be first slurried or pulped in water.

40 In general, the percent of cellulosic material by weight of the aqueous treating solution should be below 10 percent and preferably below 6.0 percent, or between about 4.0 and 6.0 percent. Good results are obtained when the de-inking solution contains about 5 to 5.5 percent by weight of paper and this value appears to be optimum. The scrap is retained in the treating solution until substantial 50 defiberization takes place. Depending upon the degree of agitation in the reactor, the time in the reactor may vary between about 10 and 50 minutes, and is usually between about 20 and 40 minutes.

55 Following treatment, the defibered material is dropped to a chest or other suitable reservoir, after which it is diluted with water to a solid content of between about 0.5 and 1.5 percent, preferably about 1.0 percent, based upon the solution weight.

60 Following dilution, the pulp is separated from the solution and washed and thickened by well known methods. The resulting pulp is then acidified to a pH of between about 4 and 6.5, preferably between about 4.5 and 5.5, thickened and then formed into a web.

65 This acidification step has been found to significantly increase the brightness of the paper produced from the

recovered pulp, and also avoids the necessity of bleaching the pulp. Moreover, it has been discovered that acidification tends to set any residual ink particles which may be present, thereby preventing such particles from coming off on the felts and rolls during the web forming step. Such residual ink particles in the past have been found to create considerable difficulty and aggravation during web forming.

The recovered stock may be blended with fresh virgin sulfate or sulfite stock, or with additional recovered stock to make cellulosic articles, such as newspaper, and so forth.

A suitable arrangement for carrying out the de-inking process is illustrated in the accompanying drawing, which is a flow sheet of the steps in a particularly suitable process in which the waste paper is added to the treating solution.

As indicated in the drawing, water from an appropriate source is charged to a suitable reactor or pulper. The reactor or pulper used in the process is equipped with a stirrer or agitator of any appropriate shape which will 20 agitate and defiber the cellulosic material. If desired, baffle plates may be attached to the interior of the reactor to assist the agitation action.

After the water has been charged to the reactor, the combined de-inking agents described herein are added and 25 agitation continued until the agents are dispersed and/or dissolved.

Wastepaper, junk, or other printed cellulosic material is then added to the reactor.

It will be understood that the sequence of addition can 30 be easily reversed with the paper being added to the dry reactor.

After a suitable period of time in the reactor, the mixture is dropped to a storage chest which is preferably equipped with a suitable agitator. If desired, water may be charged to the chest to reduce the solid content of the mixture therein. The mixture from the chest is then diluted to the solid content indicated hereinabove, and washed and thickened in a well known manner as, for example, by a 40 Lancaster three-stage washer and thickener equipped with

in the practice of the invention, such as from about 0.1% to 1% by weight of the reaction mixture of a sodium silicate such as sodium metasilicate and from about 0.1% to 1% by weight of zinc hydrosulfite or other conventional bleaching agent compatible with the basic reactants.

The following examples are exemplary of the mode of carrying out the invention:

#### EXAMPLE 1

2,000 cc. of water and the de-inking chemicals in amounts listed below are added to a standard laboratory repulping unit having an impeller which rotates at about 900 r.p.m. Thereafter 100 grams of dry newspaper is added to the unit and mixing begun.

The pulping operation is continued for 1/2 hour at room temperature. The pulp is then washed on a 60 mesh wire with a water spray until all of the ink has been removed. The pulp is next immersed in an aqueous solution of sulfur dioxide which has a pH of about 5 and permitted to stand in the solution for 10-15 minutes. The pulp is then formed into a sheet on a standard laboratory sheet mold drier.

In each example below, based on the weight of newspaper, 1.2 percent of an ethylene oxide adduct of dodecylphenol and an amount of a hydrocarbon component as listed below in Table I are employed as the de-inking chemicals.

Sodium hydroxide is added in an amount of about 0.28% by weight based on the weight of the newspaper to raise the pH of the aqueous slurry to about pH 7.5. Also added as optional ingredients are 0.41% by weight of sodium silicate and 3/8% of zinc hydrosulfite, based upon the weight of the newspaper.

The pulp thus produced, when sufficiently white in appearance can readily be handled on conventional paper making machines to produce a paper web sheet useful as newsprint.

Observations were taken on paper sheets prepared from the pulp following acidification to determine their average T.A.P.P.I. standard brightness.

TABLE I

| Example        | Newspaper treated         | Hydrocarbon component                           | Wt. percent of hydrocarbon component based on weight of newspaper | Ink remaining on sheet | Brightness             |                       |
|----------------|---------------------------|-------------------------------------------------|-------------------------------------------------------------------|------------------------|------------------------|-----------------------|
|                |                           |                                                 |                                                                   |                        | Before SO <sub>2</sub> | After SO <sub>2</sub> |
| Control A..... | Specimen.....             | None.....                                       | .....                                                             | Yes.....               | 62.7                   | 63.1                  |
| 1.....         | do.....                   | Mixture of mono-, di- & tri-chlorobenzenes..... | 0.5                                                               | No.....                | 63.0                   | 61.8                  |
| Control B..... | N.Y. Times.....           | None.....                                       | .....                                                             | Yes.....               | 63.9                   | 67.4                  |
| 2.....         | do.....                   | Same as 1.....                                  | 1.0                                                               | Small trace.....       | 63.3                   | 66.2                  |
| 3.....         | do.....                   | do.....                                         | 1.5                                                               | No.....                | 62.7                   | 65.2                  |
| 4.....         | do.....                   | Monochlorobenzene.....                          | 1.0                                                               | Small trace.....       | 66.6                   | 70.4                  |
| 5.....         | do.....                   | Dichlorobenzene.....                            | 1.0                                                               | Trace.....             | 66.7                   | 70.0                  |
| 6.....         | Bergen News (offset)..... | Monochlorobenzene.....                          | 1.0                                                               | Small trace.....       | 61.5                   | 62.0                  |
| 7.....         | do.....                   | Dichlorobenzene.....                            | 1.0                                                               | Small.....             | 60.8                   | 62.8                  |
| Control C..... | do.....                   | None.....                                       | .....                                                             | Yes.....               | 62.3                   | 63.2                  |

a 45 mesh wire screen. The pulp may be thickened to about a 5 percent solid consistency, or between about a 3 to 8 percent solid consistency in this manner. Cocurrent or counter-current washing, alone or in combination, may be used. The resulting pulp is then acidified to the pH indicated hereinabove by addition thereto of a dilute solution of a suitable acid, as for example, alum, sulfuric acid, SO<sub>2</sub>, and so forth. The resulting pulp may be finally thickened and formed into a web. The number of thickening and washing steps preceding the acidification step, it should be understood, is not critical, and the number of such treatments will be governed largely by the type of equipment employed. Also, if desired, the pulp may be bleached, 70 using a suitable bleaching agent, following acidification. Ordinarily, however, bleaching is not required. When only acidification is used, the pulp need not be, and preferably is not, washed following acidification.

Various auxiliary additives can be employed, if desired,

60 Example 3 is repeated with the exception that an ethylene oxide adduct of nonylphenol is substituted for the ethylene oxide dodecylphenol. Similar results are obtained.

#### EXAMPLE 9

65 Example 3 is repeated with the exception that diethylene glycol is substituted for ethylene glycol. Similar results are obtained.

#### EXAMPLE 10

Example 3 is repeated with the exception that propylene glycol is substituted for ethylene glycol. Similar results are obtained.

Although in the examples the de-inking agents are added to the water directly, it should be understood that the agents may also be introduced into the water in asso-

ation with the waste cellulosic material, as for example, by spraying the waste material with the de-inking agents prior to introduction of the waste newspaper into the pulper or reactor. Alternatively, water plus paper plus chemicals can be added in that order or in any order.

### EXAMPLES 11-12

The procedure of Examples 1 to 7 is repeated with the exception that the zinc hydrosulfite was omitted. The pH developed and the hydrocarbon components are shown in Table II. The specimen treated was the New York Times.

TABLE II

| x. | Hydrocarbon component   | Wt. percent of hydrocarbon component | pH  | Ink remaining on sheet | Brightness             |                       |
|----|-------------------------|--------------------------------------|-----|------------------------|------------------------|-----------------------|
|    |                         |                                      |     |                        | Before SO <sub>2</sub> | After SO <sub>2</sub> |
| 1  | Sovasol #1 <sup>1</sup> | 1.0                                  | 8.3 | None                   | 66.4                   | 70.6                  |
| 2  | Sovasol #2 <sup>2</sup> | 1.0                                  | 8.4 | None                   | 66.1                   | 71.0                  |

<sup>1</sup> Sovasol #1 is a commercial mixture of aliphatic hydrocarbons derived from petroleum and having the following characteristics:  
Specific gravity, 60/60 °F. .... gm./cc. 0.7219  
Initial boiling point. .... °F. 115  
Distillation range:  
10% .... °F. 152  
50% .... °F. 133  
90% .... °F. 226  
Dry Pt. .... °F. 246  
Aniline point. .... °F. 116  
Color. .... Water white

<sup>2</sup> Sovasol #2 is a commercial mixture of aliphatic hydrocarbons derived from petroleum and having the following characteristics:  
Specific gravity, 60/60 °F. .... gm./cc. 0.7139  
Initial boiling point. .... °F. 150  
Distillation range:  
10% .... °F. 154  
50% .... °F. 160  
90% .... °F. 172  
Dry Pt. .... °F. 191  
Aniline point. .... °F. 118  
Dimethyl sulfate value. .... 13  
Color. .... Water white

### EXAMPLE 13

The procedure of Examples 1 to 7 is repeated using the following ingredients:

|                           | Percent |
|---------------------------|---------|
| Sovasol #1                | 0.75    |
| Detergent of Examples 1-8 | 0.6     |
| Sodium hydroxide          | 1.0     |
| Sodium metasilicate       | 0.8     |
| Zinc hydrosulfite         | 0.35    |

The brightness obtained ranged from 69 to 70 after treatment with sulfur dioxide.

Although in the examples a batch, or more properly, a semi-batch process is indicated, it should be understood that the de-inking may be carried out using a continuous process, as will be obvious to those skilled in the art.

#### What is claimed:

1. In a method of de-inking waste printed paper, the improvement which comprises utilizing as the de-inking agent in aqueous solution between about 0.1 and 3.0 percent, based on the weight of the printed paper, of each of a non-ionic surface active agent and a hydrocarbon component, the non-ionic surface active agent corresponding to the formula



wherein R represents the residue of an alkyl phenol in which the total number of carbon atoms is between 7 and 14, R<sup>1</sup> represents hydrogen or lower alkyl, and n is an integer of from 2 to 100, and the hydrocarbon component being a petroleum distillate aliphatic hydrocarbon having a boiling point above about 100° F. and a melting point below about 40° F. or a liquid chlorinated monocyclic aromatic hydrocarbon having at least one chlorine atom attached to an aromatic carbon atom the weight ratio of non-ionic surface active agent to hydrocarbon component being between 10:1 and 1:10.

2. The method of claim 1 wherein the chlorinated aromatic hydrocarbon is a member selected from the

group consisting of monochlorobenzene, dichlorobenzene, trichlorobenzene and mixtures thereof.

3. A composition of matter for de-inking waste printed paper in aqueous solution which comprises a non-ionic surface active agent and a hydrocarbon component, the non-ionic surface active agent corresponding to the formula



wherein R represents the residue of an alkyl phenol in which the total number of carbon atoms is between 7 and 24, R<sup>1</sup> represents hydrogen or lower alkyl, and n is an integer of from 2 to 100, and the hydrocarbon component being a petroleum distillate aliphatic hydrocarbon having a boiling point above about 100° F. and a melting point below about 40° F. or a liquid chlorinated monocyclic aromatic hydrocarbon having at least one chlorine atom attached to an aromatic carbon atom the weight ratio of non-ionic surface active agent to hydrocarbon component being between 10:1 and 1:10.

4. The method of claim 1 wherein the non-ionic surface active agent corresponds to the formula



wherein R is the residue of alkyl phenol in which the total number of carbon atoms is between 7 and 24.

5. A process for de-inking waste printed paper which comprises pulping printed cellulosic material in an aqueous solution comprising a non-ionic surface active agent and a chlorobenzene component, the non-ionic surface active agent corresponding to the formula



wherein R represents the residue of an alkyl phenol in which the total number of carbon atoms is between 7 and 24, R<sup>1</sup> represents hydrogen or lower alkyl, and n is an integer of from 2 to 100, and the chlorobenzene component selected from the group consisting of monochlorobenzene, dichlorobenzene, trichlorobenzene and mixtures thereof, the weight ratio of non-ionic surface active agent to chlorobenzene component being between 10:1 and 1:10, the amount of printed cellulosic material being below about 10% by weight of the aqueous solution, and the amount of non-ionic detergent and chlorobenzene each being between about 0.1 and 3 percent, based upon the weight of the cellulosic material, continuing the pulping for between about 10 to 50 minutes, and separating the resulting pulp from the aqueous solution.

6. The method of claim 5 wherein the aqueous solution has an alkaline pH.

7. The method of claim 5 wherein the pH of the pulp is reduced to between about 4.0 and 6.5 following washing.

8. The method of claim 5 wherein the amount of printed paper charged to the pulper is between about 4.0 and 6.0 percent by weight of the solution.

9. The method of claim 8 wherein the amount of non-ionic detergent and chlorobenzene component is each between about 0.5 and 1.0 percent, based upon the weight of the cellulosic material.

10. A process for de-inking waste printed paper which comprises pulping printed cellulosic material in an aqueous solution having an alkaline pH comprising a non-ionic surface active agent and a petroleum distillate aliphatic hydrocarbon component, the non-ionic surface active agent corresponding to the formula



wherein R represents the residue of an alkyl phenol in which the total number of carbon atoms is between 7 and 24, R<sup>1</sup> represents hydrogen or lower alkyl, and n is an integer of from 2 to 100, the aliphatic hydrocarbon component boiling above about 100° F., the quantities by weight of each of the non-ionic surface active agents and the hydrocarbon component being from about 0.1 to

3% by weight of the cellulosic material, the amount of printed cellulosic material being below about 10% by weight of the aqueous solution, continuing the pulping for between about 10 to 50 minutes, and separating the resulting pulp from the aqueous solution.

11. A process as in claim 10 wherein the aliphatic hydrocarbon component comprises substantially saturated aliphatic hydrocarbons.

12. A process as in claim 11 wherein the reaction mixture also contains a minor amount of a sodium silicate.

13. A process as in claim 11 wherein the reaction mixture also contains a minor amount of zinc hydrosulfite.

14. A process as in claim 10 wherein the aliphatic hydrocarbon component is a mixture of aliphatic hydrocarbons, the hydrocarbon mixture being a liquid at 70°

F. and having an initial boiling point in excess of about 100° F.

15. A process in claim 14 wherein the mixture of aliphatic hydrocarbons consists essentially of saturated aliphatic hydrocarbons.

HOWARD R. CAINE, Primary Examiner

15 162—72, 74; 252—170

#### References Cited

##### UNITED STATES PATENTS

3,392,083 7/1968 Illingworth ----- 162—5

U.S. Cl. X.R,